

J. H. MELCHERS.

PROCESS FOR CONVERTING FLAX STRAW FIBER INTO PAPER PULP.

APPLICATION FILED DEC. 2, 1912.

1,162,797.

Patented Dec. 7, 1915.



WITNESSES:

J. H. Dagg et al.

Eugene L. Pindirkopf

inventor  
John H. Melchers,  
by Sonie Bain, M.A.  
Melchers

# UNITED STATES PATENT OFFICE.

JOHN HENRY MELCHERS, OF MINNEAPOLIS, MINNESOTA, ASSIGNEE TO NORTH DAKOTA STRAW PRODUCTS CO., OF McCANNA, NORTH DAKOTA, A CORPORATION OF NORTH DAKOTA.

## PROCESS FOR CONVERTING FLAX-STRAW FIBER INTO PAPER-PULP.

1,162,797.

Specification of Letters Patent.

Patented Dec. 7, 1915.

Application filed December 2, 1912. Serial No. 734,482.

To all whom it may concern:

Be it known that I, JOHN H. MELCHERS, a citizen of the United States, residing at Minneapolis, in the county of Hennepin and 5 State of Minnesota, have invented certain new and useful Improvements in Processes for Converting Flax-Straw Fiber into Paper-Pulp, of which the following is a specification.

10 My invention relates to improvements in a process for converting flax straw fiber into paper pulp.

One of the objects of my invention is to convert the exterior fiber covering of flax straw into pulp, suitable for the manufacture of paper, whereby to produce a tough smooth desirable paper.

In Figure 1, of the drawings, I have shown an arrangement of machines and devices whereby my improved process may be carried into effect. Fig. 2 is an enlarged sectional view of a straw or flax stem, showing the long silky fiber, or bast, which I segregate from the wood body-part and 25 convert into a pulp suitable, when made by my process, for the manufacture of paper.

In carrying my process of making pulp into effect, I first eliminate the dust and chaff from the straw, as much as may be, 30 and then pass it through a straw cutter 5 which cuts the straw into sections or lengths about one quarter of an inch long. It then passes on to a shaker screen 6 which removes the remaining dust. From the screen 35 6 it is passed into a grinder or shredder 7 which breaks up the woody part of the straw into fine bits and separates the fiber portion thereof into substantially the original lengths of the cut straw sections, thus fibrillating the material which I desire to convert into pulp. When the material leaves the grinder it passes on to the shaker screen 8 which sifts out the pulverized woody parts, thus leaving the fibrous material on 40 the screen. The conveyer 9 carries the fiber up to and causes it to be deposited in a "rotary" boiler or digester 10, where it is cooked under pressure in a solution of potassium carbonate ( $K_2CO_3$ ).

50 The advantages, over the usual soda process, which are obtained by my process in the

use of potassium carbonate solution are that it is more economical and that it saves the expense of caustifying as in the soda process of reclaiming, as my solution is already carbonated; that the abundance of potassium carbonate, and other potassium salts in the fiber operated upon, renders the use of potassium carbonate very desirable in extracting these salts, and furthermore, the potassium carbonate is not nearly so destructive to the fiber in the cooking of flax straw, when properly handled as the caustic alkalis after the straw has been boiled therein a sufficient length of time, and again, in the 65 process of reclaiming the potassium carbonate, less water is necessary to be evaporated as the water is eliminated which would have to be used in caustifying.

The boiling process may be effected by 70 live steam, under pressure, admitted directly into the boiler, as by steam pipe 11, or it may be circulated through suitable coils to be contained in the boiler and the pressure produced by other means,—the former 75 method, however, being preferable.

The pulp or half stuff may be emptied from the boiler 10 into a hopper, or other receptacle 12 by rotating the boiler on its axis 13—13 by means of the hand wheel 14. 80 Part of the liquid may now be carried off by the pipe 15 to the tank 18. The pulp is now taken by the conveyer 16 to a conveyer press 17, or other suitable press, whereby more of the liquid is expressed from the 85 mass. This liquid may be led off into the tank or other receptacle 18, as by means of the pipe 19, from which it may be taken for reclamation. The cooking liquid may be directly subjected to heat to evaporate the 90 water content and thereby to reclaim the potassium carbonate. This may be done without necessity of caustifying the solution preliminarily. The pulp may be now taken from the press 17, as by the conveyer 95 20, to the beater 21 where it is washed and prepared for the further treatment in the usual manner necessary prior to its formation into paper sheets.

Having described my invention what I 100 claim is:

The process of making paper pulp of

flax straw which consists in separating the woody portion of the straw from the fiber, cooking the fiber, under pressure, in a solution of potassium carbonate ( $K_2CO_3$ ), and then expressing most of the cooking liquid from the pulp and washing the pulp.

In testimony whereof I hereunto set my hand in the presence of two witnesses.

JOHN HENRY MELCHERS.

In the presence of—

SIMON MICHAEL McCANNA,  
GEO. M. McCANNA.